

[54] SOLID COMPOSITE PROPELLANT WITH AUTOCONDENSATION PRODUCT OF TRIAMINOGUANIDINIUM AZIDE AS BINDER

[75] Inventors: John J. Plomer; Harold E. Filter; George A. Lane, all of Midland, Mich.

[73] Assignee: The Dow Chemical Company, Midland, Mich.

[22] Filed: Oct. 19, 1966

[21] Appl. No.: 589,183

[52] U.S. Cl..... 149/19.1, 149/20, 149/36,  
149/38, 149/42, 149/43

[51] Int. Cl..... C06d 5/06

[58] Field of Search..... 149/18, 109, 19, 20, 36,  
149/42, 75, 83, 92, 38, 19.1, 43

[56]

References Cited

UNITED STATES PATENTS

|           |        |                    |            |
|-----------|--------|--------------------|------------|
| 2,992,908 | 7/1961 | Hedrick et al..... | 149/19.1 X |
| 2,995,432 | 8/1961 | Corley et al.....  | 149/19.1 X |
| 3,375,230 | 3/1968 | Oja et al.....     | 149/19.1 X |

Primary Examiner—Benjamin R. Padgett  
Attorney, Agent, or Firm—C. Kenneth Bjork

[57]

ABSTRACT

Propellants in which particulated solid oxidizer and metallic fuel are combined with a binder low in carbon and rich in nitrogen are disclosed. The binders are autocondensation products of triaminoguanidinium azide. An additional organic high nitrogen gas producing compound may be included.

4 Claims, No Drawings

**SOLID COMPOSITE PROPELLANT WITH  
AUTOCONDENSATION PRODUCT OF  
TRIAMINOGUANIDINIUM AZIDE AS BINDER**

This invention relates to propellants and more particularly is concerned with a novel solid propellant composition exhibiting a high specific impulse.

Conventional solid propellants based on carbon-rich binders, e.g., polyurethane, polybutadiene-acrylic acid, nitro-plasticized nitrocellulose and the like, suffer from the disadvantage that extra oxidizer must be included to oxidize the carbon. Additionally, such propellants are limited in performance by the equilibria between carbon, hydrogen, and oxygen containing compounds in the combustion products.

It is a principal object of the present invention, therefore, to provide a novel solid propellant having a binder low in carbon and rich in nitrogen which avoids these problems associated with conventional binders as well as provides a composition exhibiting a high energy content.

This and other objects and advantages readily will become apparent from the detailed description presented hereinafter.

The present invention comprises a solid propellant composition containing as a binder from about 5 to about 60 weight per cent of the autocondensation product of triaminoquanidinium azide [hereinafter referred to as Polytaz], the autocondensation products of triaminoquanidinium azide modified with from about 2 to about 20 weight per cent, based on the weight of triaminoguanidinium azide, of malononitrile [this condensation product hereinafter being referred to as Malonitaz] or cyanamide [this product being referred to herein as Cyanitaz] and mixtures thereof, from about 3 to about 65 weight per cent of a particulated solid fuel and, balance, a particulated solid oxidizer. Additionally, organic high nitrogen gas-producers such as triaminoguanidinium azide (TAZ), triaminoguanidinium hydrazinium diazide (THA), diaminoguanidinium azide, aminoguanidinium azide, hydrazinium azide hydrazinate, hydrazinium azide, ammonium azide and the like up to about 25 weight per cent of the composition weight optionally can be included in the composition. Triaminoguanidinium azide has been found to be particularly suitable.

Ordinarily the composition comprises from about 15 to about 40 weight per cent of the high nitrogen material binder, from about 8 to about 30 weight per cent of a particulated solid fuel and from about 30 to about 77 weight per cent of particulated solid oxidizer, with or without from about 5 to about 20 weight per cent of a gas producing additive.

The Polytaz binders usually have a N/C gram atom ratio of from about 2.5/1 to about 3.3/1. The malononitrile modified products (Malonitaz) ordinarily have a N/C gram atom ratio of about 3. The cyanamide modified materials (Cyanitaz) have a N/C gram atom ratio of about 5.

Conveniently these autocondensation products are

prepared by pyrolyzing triaminoguanidinium azide or mixtures of from about 80 to about 98 parts by weight triaminoguanidinium azide and from about 2 to about 20 parts by weight malononitrile or cyanamide.

5 Fuels found to be suitable for use in the present composition include, for example, light metals such as magnesium, aluminum, beryllium, light metal hydrides such as aluminum hydride, magnesium hydride, lithium aluminum hydride and the like. Aluminum, beryllium, the hydrides of these metals and mixtures thereof are preferred fuels.

The oxidizer employed in the composition usually is selected from the group consisting of ammonium perchlorate (herein designated as AP), ammonium nitrate, 15 (designated as AN), hydrazine nitroformate (designated as HNF), nitronium perchlorate (designated as NP), cyclotrimethylene-trinitramine, cyclotetramethylenetrinitramine and mixtures thereof. Ammonium perchlorate, nitronium perchlorate, hydrazine nitroformate and mixtures thereof have been found to be particularly effective oxidizers for use in the formulation of the high energy compositions. For optimum in mix compatibility and storageability when nitronium perchlorate is used ordinarily a hard, fairly non-porous polymeric surface coating is applied to the nitronium perchlorate in an amount of from about 5 to about 12 weight per cent based on the nitronium perchlorate weight.

The various solid components as used in the present 30 formulations are employed in a finely divided, particulate form as conventionally employed in solid propellant grains.

The present propellants usually are fabricated by mixing and blending the fuel, oxidizer and binder to 35 provide a substantially homogeneous blend. The formulation is cast, extruded or otherwise formed and cured to produce a solid, elastomeric propellant grain of predetermined configuration.

Satisfactory propellant grains are produced by mixing and blending at a temperature of from about 30° to 40 about 60° C. where the thermoplastic high nitrogen binder is in the liquid state, casting and curing at room temperature. Alternatively, the components can be mixed, blended and shaped or formed under pressure at room temperature thereby to provide a substantially void free, compacted propellant grain.

The following Examples will serve further to illustrate the present invention but are not meant to limit it thereto.

**EXAMPLE 1**

A number of propellant grains were formed by blending finely divided solid fuel, oxidizer and Polytaz. Each of the blends was cast into a propellant grain, cured and fired in a closed bomb. The heat energy liberated and actual specific impulse were determined for each grain. The efficiency of each grain was determined by comparing the observed specific impulse with that theoretically calculated for the composition. Table I, which follows, summarizes the data and results of this study.

Table I

| Run No. | Propellant Composition |    |    |                  |                   | Combustion Results |                               |                      |                      |                      |
|---------|------------------------|----|----|------------------|-------------------|--------------------|-------------------------------|----------------------|----------------------|----------------------|
|         | Polytaz                | Al | Be | AlH <sub>3</sub> | AP <sup>(1)</sup> | NP <sup>(2)</sup>  | ΔH <sub>r,r</sub><br>(cal./g) | Isp (obs.)<br>(sec.) | Isp (theo)<br>(sec.) | Eff.<br>(%)          |
| 1       | 35                     | 17 | —  | —                | 48                | —                  | 1435±20                       | 226                  | 273.5                | 82.7<br>(incomplete) |

Table I -Continued

| Run No. | Propellant Composition |    |    |                  |                   | Combustion Results |                              |                      |                      |             |
|---------|------------------------|----|----|------------------|-------------------|--------------------|------------------------------|----------------------|----------------------|-------------|
|         | Polytaz                | Al | Be | AlH <sub>3</sub> | AP <sup>(1)</sup> | NP <sup>(2)</sup>  | ΔH <sub>rx</sub><br>(cal./g) | Isp (obs.)<br>(sec.) | Isp (theo)<br>(sec.) | Eff.<br>(%) |
| 2       | 30                     | —  | —  | 24               | 46                | —                  | 1607±7                       | 266                  | 288.5                | 92.3        |
| 3       | 25                     | —  | —  | 30               | —                 | 45                 | 2129±79                      | 286                  | 299.9                | 95.2        |
| 4       | 10                     | —  | —  | 48               | —                 | 42                 | 2067±44                      | 284                  | 304                  | 93.5        |

<sup>(1)</sup>Ammonium perchlorate<sup>(2)</sup>Nitronium perchlorate

## EXAMPLE 2

Propellant grains were prepared by blending, casting and curing mixtures of Polytaz, aluminum hydride and ammonium perchlorate. In this preparation the binder and oxidizer were first mixed and the fuel component then blended into the composition. The grains were used as propellant in 50 gram end-burning motors. Smooth burning of the grain to completion was realized.

Composition data and motor firing results are summarized in Table II.

Table II

| Run No.          | Composition |                  |                                  | Motor Firing Results |           |               |                         |
|------------------|-------------|------------------|----------------------------------|----------------------|-----------|---------------|-------------------------|
|                  | Polytaz     | AlH <sub>3</sub> | NH <sub>4</sub> ClO <sub>4</sub> | Isp, sec.<br>(calc.) | Pa<br>psi | C*<br>ft/sec. | Burning Rate<br>in/sec. |
| (weight percent) |             |                  |                                  |                      |           |               |                         |
| 1                | 40          | 18               | 42                               | 281                  | 220       | 4368          | 0.96                    |
| 2                | 40          | 18               | 42                               | 281                  | 358       | 4841          | 1.45                    |
| 3                | 40          | 18               | 42                               | 281                  | 391       | 4708          | 2.56                    |
| 4                | 40          | 18               | 42                               | 281                  | 673       | 4947          | 1.69                    |
| 5                | 35          | 21               | 44                               | 286                  | 392       | 4776          | 1.44                    |
| 6                | 30          | 24               | 46                               | 291                  | 302       | 4890          | 1.20                    |

C\* is the characteristic exhaust velocity

## EXAMPLE 3

To evaluate the properties of the high nitrogen binders, the tensile properties of standard tensile test specimen prepared by compressing 50/50 weight per cent mixtures of Polytaz or Malonitaz with aluminum hydride were determined using an Instron tester at a cross-head speed of 2 inches/minute. The hardness was determined using a Shore Durometer tester. Additionally, a simulated propellant grain was fabricated by the same technique wherein small glass beads were incorporated into the mix to simulate particulate nitronium perchlorate oxidizer. Table III summarizes the physical properties obtained in these studies.

Table III

| Run No. | Composition                                               | Max. Tensile Strength<br>(psi) | Elongation      |      | Durometer<br>(Hardness A) |
|---------|-----------------------------------------------------------|--------------------------------|-----------------|------|---------------------------|
|         |                                                           |                                | at yield<br>(%) | max. |                           |
| 1       | Polytaz + AlH <sub>3</sub>                                | 19                             | 8               | 16   | 85                        |
| 2       | Malonitaz + AlH <sub>3</sub>                              | 240                            | 3               | 16   | 97                        |
| 3       | Malonitaz + AlH <sub>3</sub><br>+ simulated oxi-<br>dizer | 308                            | 8               | 22   | 96                        |

15 A number of propellant motor grains and strands were prepared based on Polytaz, aluminum hydride and nitronium perchlorate, ammonium perchlorate or nitronium perchlorate-ammonium perchlorate mixtures. In these studies, the nitronium perchlorate used 20 was coated with from about 5 to about 10 per cent of a proprietary polymeric composition.

The motor grains and strands were fabricated by first chilling the Polytaz binder whereupon it became brittle. The chilled binder and finely divided fuel compo-

nents were blended in a Waring Blender to provide a homogeneous, free-flowing mix having a coating of the 40 aluminum hydride fuel on the sheared polymer particles. Nitronium perchlorate was added and the resulting mixture blended. After blending, the composition was poured into a motor case or strand mold where it was pressurized to from about 100 to about 200 pounds 45 per square inch, warmed to about 30°C. and then subjected to a low pressure. The resulting cured grains or strands were substantially void free.

Bomb combustion data were carried out on a number 50 of compositions to determine the heat of explosion. The data and results from this test are summarized in Table IV.

Table IV

| Run. No.          | Composition |                  |                       |                      | ΔH <sub>rx</sub><br>(cal./gram) |
|-------------------|-------------|------------------|-----------------------|----------------------|---------------------------------|
|                   | Polytaz     | AlH <sub>3</sub> | Nitronium Perchlorate | Ammonium Perchlorate |                                 |
| (weight per cent) |             |                  |                       |                      |                                 |
| 1                 | 30          | 25               | 45                    | —                    | 1529                            |
| 2                 | 20          | 30               | 50                    | —                    | 1835                            |
| 3                 | 20          | 30               | 45                    | 5                    | 1943                            |

A pressed strand of the composition employed in Run 2 was tested to determine the burning rate. This system gave a burning rate of 1.2 inches/second at 1000 psi with a pressure exponent of 0.45.

Thirty gram end-burning motors were prepared and tested at various pressures from about 50 to about 750 psia. The compositions employed in these runs are summarized in Table V.

Table V

| Comp.<br>No. | Ingredients |                  |                                  |                                       |
|--------------|-------------|------------------|----------------------------------|---------------------------------------|
|              | Polytaz     | AlH <sub>3</sub> | NH <sub>4</sub> ClO <sub>4</sub> | NO <sub>2</sub> ClO <sub>4</sub> (NP) |
| 1            | 30          | 24               | 46                               | —                                     |
| 2            | 35          | 21               | 44                               | —                                     |
| 3            | 40          | 18               | 42                               | —                                     |
| 4            | 20          | 31               | —                                | 49                                    |

5

10

15

All motors burned smoothly with stable, normal burning being obtained at all test pressures.

## EXAMPLE 5

A number of formulations of the present invention provide high energy propellants fabricated into propellant grains. The combustion temperature and theoretical impulse of a number of such propellants were calculated. The propellant formulation data and performance results from this study are presented in Table VI which follows.

Table VI

| Run<br>No. | Propellant Composition |           |    |    |                  |                  |    |    | Results |     |                   |                              |
|------------|------------------------|-----------|----|----|------------------|------------------|----|----|---------|-----|-------------------|------------------------------|
|            | Polytaz                | Malonitaz | Al | Be | AlH <sub>3</sub> | BeH <sub>2</sub> | AP | NP | HNF     | TAZ | Comb. Temp.<br>°K | Specific Imp.<br>Isp. (sec.) |
| 1          | 10                     |           |    |    | 36               |                  |    | 54 |         |     | 4250              | 291.8                        |
| 2          | 10                     |           |    |    | 45               |                  |    | 45 |         |     | 3905              | 297.3                        |
| 3          | 15                     |           |    |    | 30               |                  |    | 55 |         |     | 4238              | 296.1                        |
| 4          | 15                     |           |    |    | 39               |                  |    | 46 |         |     | 3981              | 301.1                        |
| 5          | 20                     |           |    |    | 30               |                  |    | 50 |         |     | 4099              | 300.5                        |
| 6          | 20                     |           |    |    | 36               |                  |    | 44 |         |     | 3901              | 301.5                        |
| 7          | 25                     |           |    |    | 24               |                  |    | 51 |         |     | 4062              | 296.2                        |
| 8          | 25                     |           |    |    | 30               |                  |    | 45 |         |     | 3943              | 302.3                        |
| 9          | 25                     |           |    |    | 36               |                  |    | 39 |         |     | 3599              | 292.6                        |
| 10         | 30                     |           |    |    | 24               |                  |    | 46 |         |     | 3936              | 300.5                        |
| 11         | 30                     |           |    |    | 27               |                  |    | 43 |         |     | 3852              | 301.7                        |
| 12         | 30                     |           |    |    | 30               |                  |    | 40 |         |     | 3722              | 300.2                        |
| 13         | 35                     |           |    |    | 27               |                  |    | 38 |         |     | 3619              | 298.4                        |
| 14         | 35                     |           |    |    | 24               |                  |    | 41 |         |     | 3756              | 300.4                        |
| 15         | 35                     |           |    |    | 21               |                  |    | 44 |         |     | 3840              | 299.2                        |
| 16         | 40                     |           |    |    | 24               |                  |    | 36 |         |     | 3505              | 296.4                        |
| 17         | 40                     |           |    |    | 18               |                  |    | 42 |         |     | 3731              | 296.9                        |
| 18         | 15                     |           |    |    | 30               |                  |    | 55 |         |     | 3297              | 297.1                        |
| 19         | 15                     |           |    |    | 22               |                  |    | 63 |         |     | 3531              | 298.4                        |
| 20         | 20                     |           |    |    | 27               |                  |    | 53 |         |     | 3230              | 295.8                        |
| 21         | 20                     |           |    |    | 18               |                  |    | 62 |         |     | 3438              | 293.9                        |
| 22         | 15                     |           |    |    | 35               |                  |    | 50 |         |     | 3330              | 293.8                        |
| 23         | 15                     |           |    |    | 28               |                  |    | 57 |         |     | 3487              | 291.3                        |
| 24         | 20                     |           |    |    | 30               |                  |    | 50 |         |     | 3440              | 292.6                        |
| 25         | 20                     |           |    |    | 25               |                  |    | 55 |         |     | 3398              | 290.4                        |
| 26         | 30                     |           |    |    | 27               |                  |    | 43 |         |     | 3025              | 285.8                        |
| 27         | 30                     |           |    |    | 21               |                  |    | 49 |         |     | 3172              | 286.0                        |
| 28         | 40                     |           |    |    | 18               |                  |    | 42 |         |     | 2893              | 278.9                        |
| 29         | 20                     | 30        |    |    | 50               |                  |    |    |         |     | 3858              | 262.7                        |
| 30         | 20                     | 15        |    |    | 65               |                  |    |    |         |     | 3679              | 265.9                        |
| 31         | 30                     | 28        |    |    | 42               |                  |    |    |         |     | 3448              | 265.8                        |
| 32         | 30                     | 19        |    |    | 51               |                  |    |    |         |     | 3601              | 274.0                        |
| 33         | 30                     | 13        |    |    | 57               |                  |    |    |         |     | 3490              | 272.5                        |
| 34         | 35                     | 17        |    |    | 48               |                  |    |    |         |     | 3443              | 275.7                        |
| 35         | 40                     | 12        |    |    | 48               |                  |    |    |         |     | 3218              | 270.6                        |
| 36         | 40                     | 9         |    |    | 51               |                  |    |    |         |     | 3146              | 266.6                        |
| 37         | 40                     | 18        |    |    | 42               |                  |    |    |         |     | 3276              | 274.8                        |
| 38         | 45                     | 17        |    |    | 38               |                  |    |    |         |     | 3060              | 269.0                        |
| 39         | 30                     | 29        |    |    | 41               |                  |    |    |         |     | 4174              | 268.9                        |
| 40         | 30                     | 23        |    |    | 47               |                  |    |    |         |     | 4256              | 273.6                        |
| 41         | 30                     | 17        |    |    | 53               |                  |    |    |         |     | 4163              | 272.7                        |
| 42         | 30                     | 23        |    |    |                  |                  |    | 47 |         |     | 3316              | 274.5                        |
| 43         | 30                     | 17        |    |    | 53               |                  |    |    | 285.6   |     |                   | 280.5                        |
| 44         | 30                     | 11        |    |    | 59               |                  |    |    | 3465    |     |                   | 281.5                        |
| 45         | 15                     | 21        |    |    | 64               |                  |    |    |         |     | 3974              | 281.0                        |
| 46         | 15                     | 15        |    |    | 70               |                  |    |    |         |     | 4003              | 281.9                        |
| 47         | 20                     | 20        |    |    | 60               |                  |    |    |         |     | 3802              | 281.9                        |
| 48         | 20                     | 14        |    |    | 66               |                  |    |    |         |     | 3907              | 284.1                        |
| 49         | 25                     | 12        |    |    | 63               |                  |    |    |         |     | 3769              | 286.0                        |
| 50         | 25                     | 18        |    |    | 57               |                  |    |    |         |     | 3710              | 285.4                        |
| 51         | 30                     | 19        |    |    | 51               |                  |    |    |         |     | 3506              | 280.8                        |
| 52         | 30                     | 13        |    |    | 57               |                  |    |    |         |     | 3712              | 290.7                        |
| 53         | 30                     | 7         |    |    | 63               |                  |    |    |         |     | 3495              | 281.8                        |
| 54         | 35                     | 12        |    |    | 53               |                  |    |    |         |     | 3587              | 292.6                        |
| 55         | 40                     | 13        |    |    | 47               |                  |    |    |         |     | 3318              | 289.2                        |
| 56         | 40                     | 7         |    |    | 53               |                  |    |    |         |     | 3304              | 283.3                        |
| 57         | 45                     | 9         |    |    | 46               |                  |    |    |         |     | 3277              | 289.3                        |
| 58         | 30                     | 22        |    |    | 48               |                  |    |    |         |     | 3932              | 279.4                        |
| 59         | 30                     | 16        |    |    | 54               |                  |    |    |         |     | 4461              | 289.9                        |
| 60         | 30                     | 13        |    |    | 57               |                  |    |    |         |     | 4370              | 286.8                        |
| 61         | 30                     | 10        |    |    | 60               |                  |    |    |         |     | 4188              | 282.0                        |
| 62         | 40                     | 16        |    |    | 44               |                  |    |    |         |     | 3862              | 290.1                        |
| 63         | 40                     | 13        |    |    | 47               |                  |    |    |         |     | 4120              | 296.3                        |
| 64         | 40                     | 10        |    |    | 50               |                  |    |    |         |     | 4081              | 293.6                        |
| 65         | 50                     | 10        |    |    | 40               |                  |    |    |         |     | 3750              | 299.1                        |
| 66         | 50                     | 13        |    |    | 37               |                  |    |    |         |     | 3502              | 290.1                        |
| 67         | 50                     | 7         |    |    | 43               |                  |    |    |         |     | 3744              | 296.0                        |
| 68         | 60                     | 7         |    |    | 33               |                  |    |    |         |     | 3309              | 291.9                        |
| 69         | 60                     | 4         |    |    | 36               |                  |    |    |         |     | 3197              | 283.5                        |
| 70         | 60                     | 10        |    |    | 30               |                  |    |    |         |     | 3082              | 288.1                        |

Table VI—Continued

| Run No. | Propellant Composition |           |      |      |                  |                  |      |    | Results |      |                |                           |
|---------|------------------------|-----------|------|------|------------------|------------------|------|----|---------|------|----------------|---------------------------|
|         | Polytaz                | Malonitaz | Al   | Be   | AlH <sub>3</sub> | BeH <sub>2</sub> | AP   | NP | HNF     | TAZ  | Comb. Temp. °K | Specific Imp. Isp. (sec.) |
| 71      | 30                     |           |      | 16   |                  |                  |      |    | 54      |      | 3447           | 288.2                     |
| 72      | 30                     |           |      | 10   |                  |                  |      |    | 60      |      | 3599           | 299.6                     |
| 73      | 30                     |           |      | 7    |                  |                  |      |    | 63      |      | 3489           | 293.8                     |
| 74      | 30                     |           |      | 4    |                  |                  |      |    | 66      |      | 3354           | 285.1                     |
| 75      | 20                     |           |      | 16   |                  |                  |      |    | 64      |      | 3706           | 295.1                     |
| 76      | 20                     |           |      | 10   |                  |                  |      |    | 70      |      | 3777           | 296.7                     |
| 77      | 40                     |           |      | 7    |                  |                  |      |    | 53      |      | 3280           | 291.8                     |
| 78      | 40                     |           |      | 13   |                  |                  |      |    | 47      |      | 3248           | 287.4                     |
| 79      | 18                     |           |      | 11.4 |                  |                  | 50.6 |    |         | 20   | 3553           | 294.1                     |
| 80      | 23                     |           |      | 10.5 |                  |                  | 46.5 |    |         | 20   | 3417           | 294.1                     |
| 81      | 30                     |           |      | 11.1 |                  |                  | 48.9 |    |         | 10   | 3477           | 293.8                     |
| 82      | 35                     |           |      | 11   |                  |                  | 47.5 |    |         | 65   | 3417           | 293.0                     |
| 83      | 20                     |           |      |      | 17               | 63               |      |    |         |      | 3441           | 312.6                     |
| 84      | 20                     |           |      |      | 23               | 57               |      |    |         |      | 3214           | 319.5                     |
| 85      | 20                     |           |      |      | 29               | 51               |      |    |         |      | 2823           | 327.2                     |
| 86      | 20                     |           |      |      | 32               | 48               |      |    |         |      | 3004           | 318.4                     |
| 87      | 30                     |           |      |      | 19               | 51               |      |    |         |      | 3136           | 313.1                     |
| 88      | 30                     |           |      |      | 25               | 45               |      |    |         |      | 2820           | 319.5                     |
| 89      | 30                     |           |      |      | 28               | 42               |      |    |         |      | 2845           | 310.7                     |
| 90      | 20                     |           |      | 22   |                  |                  | 58   |    |         |      | 3972           | 322.3                     |
| 91      | 20                     |           |      | 31   |                  |                  | 49   |    |         |      | 3239           | 328.4                     |
| 92      | 20                     |           |      | 34   |                  |                  | 46   |    |         |      | 3369           | 324.5                     |
| 93      | 30                     |           |      | 25   |                  |                  | 45   |    |         |      | 3390           | 323.8                     |
| 94      | 30                     |           |      | 31   |                  |                  | 39   |    |         |      | 2759           | 336.7                     |
| 95      | 30                     |           |      | 34   |                  |                  | 36   |    |         |      | 3139           | 316.6                     |
| 96      | 20                     |           |      | 15   |                  |                  | 65   |    |         |      | 3414           | 318.8                     |
| 97      | 20                     |           |      | 21   |                  |                  | 59   |    |         |      | 3209           | 319.1                     |
| 98      | 30                     |           |      | 14   |                  |                  | 56   |    |         |      | 3171           | 313.5                     |
| 99      | 30                     |           |      | 20   |                  |                  | 50   |    |         |      | 3012           | 310.6                     |
| 100     | 25                     |           | 14.3 |      |                  |                  | 40.7 |    |         | 20   | 3940           | 286.9                     |
| 101     | 30                     |           | 13   |      |                  |                  | 37   |    |         | 20   | 3765           | 286.5                     |
| 102     | 35                     |           | 14.3 |      |                  |                  | 40.7 |    |         | 10   | 3924           | 286.3                     |
| 103     | 40                     |           | 13   |      |                  |                  | 37   |    |         | 10   | 3740           | 285.8                     |
| 104     | 45                     |           | 12.4 |      |                  |                  | 32.6 |    |         | 10   | 3506           | 283.2                     |
| 105     | 35                     |           |      | 11   |                  |                  | 44   |    |         | 10   | 3896           | 297.0                     |
| 106     | 40                     |           |      | 10   |                  |                  | 40   |    |         | 10   | 3727           | 298.2                     |
| 107     | 45                     |           |      | 9    |                  |                  | 36   |    |         | 10   | 3538           | 297.1                     |
| 108     | 30                     |           |      | 3    | 12               | 55               |      |    |         |      | 3081           | 299.5                     |
| 109     | 30                     |           |      | 5    | 20               | 45               |      |    |         |      | 2887           | 309.7                     |
| 110     | 30                     |           |      | 6    | 24               | 40               |      |    |         |      | 2823           | 307.3                     |
| 111     | 40                     |           |      | 2    | 8                | 50               |      |    |         |      | 2850           | 285.9                     |
| 112     | 40                     |           |      | 5    | 20               | 35               |      |    |         |      | 2749           | 299.8                     |
| 113     |                        | 10        |      | 36   |                  |                  | 54   |    |         |      | 4232           | 298.1                     |
| 114     |                        | 10        |      | 45   |                  |                  | 45   |    |         |      | 3869           | 296.4                     |
| 115     |                        | 15        |      | 33   |                  |                  | 52   |    |         |      | 4151           | 298.8                     |
| 116     |                        | 15        |      | 42   |                  |                  | 43   |    |         |      | 3753           | 294.6                     |
| 117     |                        | 20        |      | 30   |                  |                  | 50   |    |         |      | 4048           | 298.2                     |
| 118     |                        | 20        |      | 36   |                  |                  | 44   |    |         |      | 3819           | 297.6                     |
| 119     |                        | 20        |      | 39   |                  |                  | 41   |    |         |      | 3619           | 291.5                     |
| 120     |                        | 25        |      | 27   |                  |                  | 48   |    |         |      | 3953           | 297.9                     |
| 121     |                        | 25        |      | 30   |                  |                  | 45   |    |         |      | 3851           | 298.3                     |
| 122     |                        | 25        |      | 33   |                  |                  | 42   |    |         |      | 3698           | 295.4                     |
| 123     |                        | 30        |      | 24   |                  |                  | 46   |    |         |      | 3844           | 296.3                     |
| 124     |                        | 30        |      | 27   |                  |                  | 43   |    |         |      | 3735           | 296.4                     |
| 125     |                        | 30        |      | 30   |                  |                  | 40   |    |         |      | 3561           | 292.3                     |
| 126     | 10                     |           |      | 30   |                  |                  | 50   |    | 10      | 4118 | 300.2          |                           |
| 127     | 10                     |           |      | 33   |                  |                  | 52   |    | 5       | 4195 | 299.6          |                           |
| 128     | 10                     |           |      | 42   |                  |                  | 43   |    | 5       | 3837 | 298.0          |                           |
| 129     | 10                     |           |      | 39   |                  |                  | 41   |    | 10      | 3765 | 298.2          |                           |
| 130     |                        | 10        |      | 33   |                  |                  | 52   |    | 5       | 4174 | 299.6          |                           |
| 131     |                        | 10        |      | 39   |                  |                  | 46   |    | 5       | 3959 | 300.0          |                           |
| 132     |                        | 10        |      | 42   |                  |                  | 43   |    | 5       | 3799 | 296.8          |                           |
| 133     |                        | 10        |      | 30   |                  |                  | 50   |    | 10      | 4091 | 299.8          |                           |
| 134     |                        | 10        |      | 36   |                  |                  | 44   |    | 10      | 3892 | 300.8          |                           |
| 135     |                        | 10        |      | 27   |                  |                  | 48   |    | 15      | 4020 | 300.3          |                           |
| 136     |                        | 10        |      | 33   |                  |                  | 42   |    | 15      | 3821 | 301.2          |                           |
| 137     |                        | 10        |      | 24   |                  |                  | 46   |    | 20      | 3944 | 300.3          |                           |
| 138     |                        | 10        |      | 30   |                  |                  | 40   |    | 20      | 3745 | 300.9          |                           |
| 139     |                        | 10        |      | 33   |                  |                  | 37   |    | 20      | 3558 | 295.5          |                           |

In a manner similar to that described for the preceding Examples, solid propellant compositions can be formulated using particulate fuels and oxidizers, gas producing additives, and binder components set forth herein. These can be used in various combinations within the disclosed ranges.

Various modifications can be made in the present invention without departing from the spirit or scope thereof for it is understood that we limit ourselves only as defined in the appended claims.

65

We claim:

1. A solid propellant composition comprising on a weight basis

- from about 5 to about 60 per cent of a binder member selected from the group consisting of the autocondensation product of triaminoguanidinium azide, the autocondensation product of triaminoguanidinium azide modified with from about 2 to about 20 weight per cent malononitrile, the autocondensation product of triaminoguanidinium azide modified with from about 2 to about 20 weight per cent cyanamide and mixtures thereof,
- from about 3 to about 65 weight per cent of a particulated solid fuel, and
- balance a particulated solid oxidizer.

2. The solid propellant composition as defined in claim 1 wherein on a weight basis the binder ranges from about 15 to about 40 per cent, the particulated solid fuel is from about 8 to about 30 per cent, said fuel being a member selected from the group consisting of aluminum, beryllium, aluminum hydride, beryllium hydride and mixtures thereof, and, the particulate solid oxidizer ranges from about 30 to about 77 per cent, said oxidizer being a member selected from the group consisting of ammonium perchlorate, nitronium per-

chlorate, hydrazine nitroformate and mixtures thereof.

3. The composition as defined in claim 1 and including, based on the total composition weight, up to about 25 per cent of an organic high nitrogen gas producing compound.

4. The composition as defined in claim 2 and including from about 5 to about 20 weight per cent triaminoguanidinium azide.

\* \* \* \* \*

UNITED STATES PATENT OFFICE  
CERTIFICATE OF CORRECTION

Patent No. 3,844,855 Dated October 29, 1974  
Inventor(s) John J. Plomer, Harold E. Filter, George A. Lane

It is certified that error appears in the above-identified patent and that said Letters Patent are hereby corrected as shown below:

Table VI, Run No. 43 and 44 should read as follows under the indicated headings :

| Run No. | NP | HNF | TAZ | Comb. Temp.<br>°K | Specific Imp.<br>Isp. (sec.) |
|---------|----|-----|-----|-------------------|------------------------------|
| 43      |    | 53  |     | 3555              | 285.6                        |
| 44      |    | 59  |     | 3465              | 281.5                        |

Signed and sealed this 18th day of February 1975.

(SEAL)

Attest:

RUTH C. MASON  
Attesting Officer

C. MARSHALL DANN  
Commissioner of Patents  
and Trademarks